

## UNITED STATES PATENT OFFICE

2,357,275

CORROSION INHIBITION COATING  
COMPOSITION

Aaron Wachter, San Francisco, Calif., assignor to  
Shell Development Company, San Francisco,  
Calif., a corporation of Delaware

No Drawing. Application July 22, 1941,  
Serial No. 403,533

5 Claims. (Cl. 44—72)

The present invention relates to corrosion prevention coatings and more specifically to coatings for preventing corrosion of metal surfaces by the water often associated in small amounts with water-immisile liquids.

In the storage and handling of various water-immisile liquid materials, particularly hydrocarbons, it is often necessary both to transport and/or to store such materials in metal containers, as in steel drums or tanks and the like. Since these materials often contain varying amounts of water in solution or in suspension, which may separate due to temperature changes for example, internal corrosion of the container by the water almost always occurs to a greater or lesser degree. This problem is particularly serious when gasoline is under consideration. In spite of all reasonable and practicable precautions during the manufacture of gasoline, when the same is stored in drums or tanks for a period, especially as is so often practiced in handling aviation gasoline, an appreciable amount of water separates and will be found as a film or in minute droplets on the container walls or even in small pools in the bottom of the container. This of course brings about ideal conditions for corrosion and consequent damage to the container as well as the even more serious contamination of the gasoline or similar product stored within the container.

It is to be clearly understood that the corrosion inhibiting coating described below is intended for use only in those cases in which relatively small quantities of water come in contact with the surfaces to be protected, as distinguished from primarily aqueous systems, such as water tanks, etc.

As a result of the above described corrosion, it has become necessary for manufacturers and shippers of such products to apply various internal coatings to the walls of such containers or to add corrosion inhibitors of one type or another to the product being stored.

It is an object of the present invention to provide an improved internal coating for containers which are to be used as described above. It is a further object of this invention to provide an internal coating which will both prevent corrosion and remove to a large extent any corrosion products already present in material which may be transferred to containers protected with the hereinafter described improved coating. Another object is to provide an internal container coating which will prevent contact between the container walls and the material stored therein, thus preventing corrosion of the container by materials which may be dissolved in the stored material, such as organic acids and sulfur compounds. Further objects are to supply a coating which is inexpensive, easily applied and removed, and

which does not contaminate in any way materials stored in containers protected by the same.

Broadly, the present improved coating comprises a hydrocarbon insoluble, water-soluble mucilaginous material, a plasticizer if necessary, and sodium nitrate. By mucilaginous material is meant those materials which either alone or in the presence of a suitable plasticizer provide a continuous, pliable film when applied in solution and the solvent removed therefrom. Most of the proteins and carbohydrates of animal and vegetable origin and products derived therefrom fall within the limits of this definition. For example, pure grades of the following types of compounds and mixtures of the same will be found suitable: proteins, albuminoids, glues, gelatins, phosphoproteins, caseins, sugars, starches, dextrans, gums and cellulose derivatives. More specifically, the following compounds are among those suitable as the mucilaginous base material in the presently disclosed coating: corn starch (partially hydrolyzed), molasses, gum arabic, agar-agar, dextrin, pectin, barley sugar, caramel, xylan, wheat gluten and gum tragacanth.

As a specific example and in a preferred embodiment of the invention, the following composition has been found especially satisfactory:

| Per cent by weight, approximately |    |  |
|-----------------------------------|----|--|
| Dextrin                           | 60 |  |
| Glycerin                          | 30 |  |
| Inhibitor                         | 10 |  |

The above material is applied preferably as an approximately 40% water solution and the water thereafter is permitted to evaporate or is removed by heating the container at a temperature not substantially exceeding 300° F., for a period of time not substantially exceeding 10 minutes. The resulting coating is pliable, tacky, water soluble and hydrocarbon insoluble. It is non-poisonous, odorless and may be easily removed by the usual drum washing processes. Under prolonged severe testing conditions containers protected with the above coating and containing gasoline evidenced no traces of internal corrosion; unprotected containers subjected to the identical tests were severely corroded and their contents so thoroughly contaminated as to be practically valueless without recovery treatment.

The coating is preferably applied by spraying a quantity of the 40% solution into the container and drawing off any excess before drying, although other methods such as brush application in large storage tanks may be utilized if desired.

In any case, application conditions should be adjusted to provide at least approximately 3 milligrams of dehydrated coating per square inch of surface to be protected. A usually satisfactory coating is attained if from 1 to 2 fluid ounces of the 40% solution are sprayed into a 55 gallon

drum, in a manner to cover all internal surfaces, the drum then being subjected to a temperature of about 250° F. for approximately 5 minutes.

This process may be easily included in the commonly employed drum cleaning treatment where-in dirty drums are washed with a hot alkaline solution, rinsed, steamed, dried and heated prior to painting the exterior surfaces. After the drums have been dried, the above described coating may be applied and the drums passed on to the heating stage in the usual manner. The washing steps will remove all traces of a previous protective coating if such has been applied.

Although glycerin is the preferred plasticizer for use in the present coating, glycol and other hydrocarbon insoluble polyhydric alcohols, glycerin polymers, amines, hydroxy amines, hydroxy ethers, and similar materials which have known plasticizing properties will also usually be found satisfactory.

The amounts of the various components of the coating may be varied within certain limits without deleterious effects. The formula given above, i. e. base, plasticizer and inhibitor in the approximate proportions of 60:30:10 has been found to be generally satisfactory for normal conditions of service and in fact includes an appreciable safety factor in the quantity of inhibitor incorporated. Sodium nitrite, for example, is known to be an efficient inhibitor at concentrations as low as .02%; however, in view of the relatively small quantities actually used in employing the preferred formula (1.5 grams in a 55 gallon drum) and in order to obviate completely any danger of localized corrosion due to the possibility of a relatively large pool of water occurring in the container, it is considered preferable to employ a reasonable excess of inhibitor. The relative proportions of base and plasticizer used will of necessity vary with the specific materials utilized. In the case where dextrin is used as a base and glycerin as a plasticizer, from approximately 40% to 85% dextrin, the balance being glycerin and inhibitor (from .02 to 10%), has been found satisfactory.

As has been mentioned above, the inhibitor coating is applied in solution, water being the preferred solvent. A solution containing 40% by weight of the inhibitor coating has been found preferable for general use. However, solutions containing from 15% to 75% may be used, depending upon the thickness of coating desired and the conditions under which the solvent is to be removed.

When using other materials than dextrin as the mucilaginous base, the relative quantities of the various components may require modification. For example, a suitable coating may be formulated using the following materials in the proportions noted:

|                  | Per cent by weight,<br>approximately |
|------------------|--------------------------------------|
| Arrowroot starch | 5                                    |
| Glycerin         | 85                                   |
| Sodium nitrite   | 10                                   |

In this formula, the quantity of starch may be

varied from approximately .5% by weight to approximately 10% by weight. Not less than approximately 60% by weight of glycerin should be used, however, or an unsatisfactory coating will result. This composition is preferably applied in an approximately 50% solution in water.

Another coating which has been found suitable is formulated as follows:

|                      | Per cent by weight,<br>approximately |
|----------------------|--------------------------------------|
| Liquid glue (animal) | 80                                   |
| Glycerin             | 10                                   |
| Sodium nitrite       | 10                                   |

The above is preferably applied in an approximately 30% solution in water. In many instances, depending primarily upon the particular source from which the liquid glue is derived, the glycerin may be eliminated from this formula, using instead a composition comprising not less than 0.02% and preferably about 10% by weight of sodium nitrite and the balance liquid glue. This coating can be most advantageously applied in an approximately 40% solution in water.

I claim as my invention:

1. A water-soluble corrosion inhibiting coating composition suitable for protecting metal surfaces in contact with hydrocarbons containing small amounts of water against corrosion comprising from 40% to 85% by weight of dextrin, at least .02% by weight sodium nitrite and the balance a water-soluble polyhydric alcohol.

2. A water-soluble corrosion inhibiting coating composition suitable for protecting metal surfaces in contact with hydrocarbons containing small amounts of water against corrosion comprising approximately 60% by weight of dextrin, approximately 30% by weight of a water-soluble polyhydric alcohol and the balance sodium nitrite, said coating having a pH of at least 6 in water solution.

3. A water-soluble corrosion inhibiting coating composition suitable for protecting metal surfaces in contact with hydrocarbons containing small amounts of water against corrosion comprising about 5-80% by weight of a water-soluble hydrocarbon-insoluble mucilaginous base, about 10-85% by weight of a water-soluble polyhydric alcohol, and about .02 to 10% by weight of sodium nitrite.

4. A water-soluble corrosion inhibiting coating composition suitable for protecting metal surfaces in contact with hydrocarbons containing small amounts of water against corrosion comprising about 5-80% by weight of a water-soluble hydrocarbon-insoluble mucilaginous base, about 10-85% by weight of a water-soluble polyhydric alcohol, and at least .02% by weight of sodium nitrite.

5. A water-soluble corrosion inhibiting coating composition suitable for protecting metal surfaces in contact with hydrocarbons containing small amounts of water against corrosion comprising from 40% to 85% by weight of dextrin, at least .02% by weight of sodium nitrite and the balance glycerin.

AARON WACHTER.